

## UNITED STATES PATENT OFFICE.

FERDINAND MÜNZ, OF FECHENHEIM-ON-THE-MAIN, GERMANY, ASSIGNOR TO LEO-FOLD CASSELLA & CO., GESELLSCHAFT MIT BESCHRANKTER HAFTUNG, A CORPORATION OF GERMANY.

PROCESS FOR DYEING WITH DYESESTUFFS OR DYESESTUFFS-PRODUCING BODIES  
INSOLUBLE OR SPARINGLY SOLUBLE IN WATER.

No Drawing.

Application filed September 3, 1924. Serial No. 735,690.

*To all whom it may concern:*

Be it known that I, FERDINAND MÜNZ, a citizen of the Austrian Republic, residing at Fechenheim-on-the-Main, Germany, have invented a Process for Dyeing with Dye-stuffs or Dyestuff-Producing Bodies Insoluble or Sparingly Soluble in Water, of which the following is a full description.

Numerous dyestuffs and dyestuff-producing bodies hitherto could not be employed for dyeing the various fibres, because their insufficient solubility presented an obstacle.

It has now been found, that a great number of these bodies can be made suitable for dyeing when mixed with organic solvents and soaps, by means of which a sufficient solubility, allowing them to be dyed in an aqueous bath is attained.

Ordinary soaps, as well as sulfonated products, Turkey-red oils, monosolvol and the like may be employed, as organic solvents benzene and its homologues, hydrated carbohydrates, chlorocarbohydrates and similar bodies, as far as they exercise a dissolving action on the respective dyestuffs and dyestuff-producing bodies insoluble in water. A slight addition of alkalies as soda and ammonia enhances the solubility of the respective products.

The carrying into execution and application of the process is explained by the following examples:

*Example 1.*

2% dimethylamidoazobenzene, 4% Turkey-red oil, 4% solvent naphtha, 0.4% soda, of the weight of the silk to be dyed are

boiled up with 40-50 times the quantity of water and added to the dyebath heated to 80-85° C. (176-185° F.), in which the silk is treated for about  $\frac{3}{4}$  hour; the bath is well exhausted, and a clear yellow obtained.

*Example 2.*

Acetate silk is dyed with 3% of the dye-stuff derived from o-anisidine-alphanaphthylamine, 8% common curd soap, 5% tetraline, 1.5% soda as indicated in example 1, however at a temperature of 60-65° C. (140-149° F.), diazotized on the fibre, and developed with 2,3-oxynaphthoic acid. A deep black is obtained.

*Example 3.*

The acetate silk is treated with 0.5% dianisidine, 2% soap, 1.5% tetraline, 0.5% soda, as indicated in example 2, likewise diazotized on the fibre, and developed with 2,3-oxynaphthoic acid. A clear blue is obtained.

The great variety of insoluble azo dye-stuffs and components of same, as well as other insoluble products may be employed in an analogous manner.

*Claim:*

A process of dyeing with dyestuffs and dyestuff-producing bodies insoluble or sparingly soluble in water, by applying them together with organic solvents not miscible with water and soaps in an aqueous bath.

In witness whereof I have hereunto signed my name this 20th day of August 1924.

FERDINAND MÜNZ.